

## UNITED STATES PATENT OFFICE

2,485,150

## MINERAL OIL COMPOSITIONS

Frank J. Glavis, Elkins Park, and Harry T. Neher,  
Bristol, Pa., assignors to Röhm & Haas Company,  
Philadelphia, Pa., a corporation of Delaware

No Drawing. Application January 21, 1947,  
Serial No. 723,462

3 Claims (Cl. 252—33.4)

1

This invention deals with compositions of matter comprising a major proportion of a mineral oil and minor proportions of an oil-soluble petroleum sulfonate and a water-insoluble, oil-miscible araliphatic polyether alcohol of the formula



wherein R is an alkyl group of four to twelve carbon atoms. These compositions are useful as slushing oils, lubricating oils, and the like.

It has already been proposed to add petroleum sulfonates to mineral oils to impart to the resulting compositions anti-corrosive properties or detergent action. Actual, practical results have varied greatly. In many instances, the protective value of the compositions has been insufficient at moderate concentrations of petroleum sulfonate. While larger proportions of such sulfonate have then been tried, the resulting compositions have not been proportionately more effective and disadvantageous properties have been thus developed. While compositions have been devised which give sufficient protection for slight or moderate exposure to corrosive conditions, these often fail when conditions become slightly more severe. This is particularly true in thin film applications. Furthermore, there has been considerable variation in results from a given formulation. Often it is desirable or even necessary that the composition not only protect metals from corrosion but also provide safe and efficient lubrication. Few compositions of the art have had this desirable combination of properties. It is readily attained, however, by practicing this invention which, at the same time, corrects many of the shortcomings and deficiencies of compositions of the prior art.

It is an object of this invention to provide compositions of improved anti-corrosive action. It is an object to provide compositions which supply a high degree of protection of metal surfaces, particularly ferrous surfaces, against corrosion from moisture and aqueous solutions of electrolytes. It is an object to provide compositions in which a given amount of an oil-soluble petroleum sulfonate is rendered more effective. It is an object to provide compositions in which relatively small amounts of petroleum sulfonates are rendered effective. It is also an object to provide lubricating compositions which, when used on metal surfaces, afford a high degree of protection against corrosion.

These and other objects are accomplished by this invention wherein mineral oils are improved

2

by the addition of oil-soluble petroleum sulfonates and an alkylphenoxyethoxyethoxyethanol. The compositions of this invention provide excellent protection of metals against moisture and many aqueous solutions, whether used in thick or in thin film applications, and at the same time may serve as lubricants for the surfaces of the metal.

An essential component of the compositions of this invention is an oil-soluble petroleum sulfonate. This may be an alkali or alkaline earth salt, including the lithium, sodium, potassium, calcium, strontium, and barium salts of the hydrocarbon sulfonates prepared by the treatment of petroleum oils with sulfuric acid followed, for example, by treatment with a base of the metal. While the alkali or alkaline earth sulfonates are those most commonly used and most readily available, petroleum sulfonates of other metals may be used if they are soluble in the particular mineral oil selected to an extent of 1% to 10%. The most effective sulfonates are those of moderately high molecular weight. These are usually regarded as having molecular weights of about five hundred to about seven hundred. Yet any of the oil-soluble petroleum sulfonates may be used which have molecular weights from about four hundred to about one thousand, the range of five hundred to seven hundred being preferred. The oil-soluble metal sulfonates may be used in amounts from 0.5% to 7.5%, with concentrations of 1% to 5% being most desirable for a balance of efficiency and economy. While more than 7.5% may be used in conjunction with an alkylphenoxyethoxyethanol in a petroleum oil, there is usually no practical advantage gained thereby except for the preparation of concentrates which are diluted before use. Since it is generally considered desirable to use as small amounts of additives as will produce desired results with some factor of safety, the amount of petroleum sulfonate actually used should depend on the intended application and the conditions there to be met.

The sulfonate may be used at a concentration which, if it were the sole additive, would not provide an acceptable degree of protection to metals. Upon addition of an alkylphenoxyethoxyethoxyethanol in small amount, however, the resulting composition gains greatly in effectiveness. Yet this latter compound as a sole additive may actually promote corrosion. It is desirably used more or less in proportion to the amount of sulfonate taken. The practical limits are from 0.05% up

to 3% of an alkylphenoxyethoxyethoxyethanol which is preferably used in an amount no greater than the amount of petroleum sulfonate being used.

The polyether alcohols which are used fall within the formula



where R is an alkyl group of four to twelve carbon atoms. Thus, R may be butyl, amyl, hexyl, heptyl, octyl, nonyl, decyl, undecyl, or dodecyl in straight or branched chain arrangement with the group being normal iso, secondary, or tertiary and with the alkyl group in ortho-meta, or para positions. When this group is tertiary, particularly interesting compounds are at hand from the point of view of economy and effectiveness. The phenyl nucleus may contain more than one hydrocarbon constituent, as in the case of the nucleus from alkylated cresols or xylenols or alkylated ethylphenol or other alkylated hydrocarbon-substituted phenols, as in the case of groups derived from poly-hydrocarbon-substituted phenols such as tert.-butylphenylphenol or butyl cyclohexylphenol. The essential requirement of the alkylated phenyl group is that it impart ready oil-solubility and be free from polar or reactive groups.

As is known, compounds of the above formula are prepared from alkylated phenols by reaction with three moles of ethylene oxide or by reaction with a triethylene halohydrin in the presence of a base.

In addition to an oil-soluble petroleum sulfonate and the oil-soluble ether alcohols above defined, there may be used in the compositions of this invention one or more additives providing special properties, such as antioxidants, oiliness agents, pour point depressants, viscosity index improvers, extreme pressure agents, thickening agents, including petrolatum and waxes, and the like.

The beneficial effects of the combination of sulfonate and the above-defined ether alcohols have been established with oils from paraffinic, naphthenic, and asphaltic stocks, and combinations thereof. Furthermore, oils have been used which were refined by distillation, by extraction, and by a combination of distillation and extraction. Oils have been studied varying in viscosity from about one hundred seconds to fifteen hundred seconds Saybolt at 100° F. and varying in viscosity index from zero to well over one hundred. In every case, the addition of an alkylphenoxyethoxyethoxyethanol has markedly improved the properties of a petroleum sulfonate in oil.

The following examples show typical results obtained with compositions of this invention:

#### Example 1

A series of alkylphenyl ether alcohols was prepared having one, three, five, eight, and thirteen ether groups, the alkyl group being octyl. There was also prepared a 5% solution of a sodium petroleum sulfonate of a molecular weight of about 450 in an S. A. E. 10 lubricating oil prepared by solvent extraction of a fraction from mid-continent crude. This oil had a viscosity index of 115. Solutions were made with one per cent of each of these ether alcohols in the 5% sulfonate solution. These solutions were then tested on standard steel panels which were hung in a cabinet

at 120° F. maintained at 100% relative humidity. Panels coated with the 5% sulfonate solution without an ether alcohol were rusted within twenty-nine hours. The panels coated with the solution containing sulfonate and the compound having thirteen ether groups were rusted within seventeen hours. The panels with the sulfonate and ether alcohols of eight and five ether groups, respectively, were rusted within two days' time. 10 Panels with the sulfonate and alcohol with a single ether group rusted within about three days. The panels with the sulfonate and the compound with three ether groups were intact at the end of ten days, when the tests were discontinued.

#### Example 2

In an oil prepared from mid-continent stock, having a viscosity index of 116 as a result of solvent extraction and having a viscosity of 530 seconds Saybolt at 100° F., there were dissolved 20 0.1% of a thiophosphate as an antioxidant and 1.5% of a calcium petroleum sulfonate of relatively low molecular weight. Panels coated with this mixture were rusted in the humidity cabinet at 120° F. within three hours after initial exposure. To a portion of this solution there was added one per cent of tert.-butylphenoxyethoxyethoxyethanol; and this mixture was applied to steel panels, which were exposed to a saturated atmosphere at 120° F. No rust appeared until after sixty-eight hours. This composition was found to be a good, stable, anti-corrosive engine oil with detergent properties.

#### Example 3

35 A 3% solution of a sodium petroleum sulfonate of a molecular weight of about five hundred was made in the oil described in Example 2. This prevented corrosion of steel panels in a moisture saturated atmosphere at 120° F. for four days. 40 Addition to this solution of 1% of diisobutylphenoxyethoxyethoxyethanol greatly increased the protective value of the composition, no rust appearing on steel panels in a full week, at which time the tests were discontinued. During the 45 same period, tests were run with solutions of the same sulfonate with the same oil, to which was added only 0.25% of the same ether alcohol in one case and 0.5% in another case. Both of these 50 compositions effectively prevented rusting for over 168 hours.

#### Example 4

A series of solutions was made in which a high-grade petroleum sulfonate of a molecular weight about five hundred, regarded in the trade as a very effective rust-preventive agent, was dissolved in a mid-continent S. A. E. 30 motor oil to give solutions containing from 2% to 10% of the sulfonate. Steel panels coated with this series of sulfonate solutions all rusted in seventy to eighty hours when placed in the humidity cabinet referred to in Example 1. Addition of 0.1% of tert.-octylphenoxyethoxyethoxyethanol to the 2% solution increased the protective period to over ninety hours, while addition of 0.1% to the 7% solution increased this period to over 150 hours. Addition of 0.2% of this compound to the 5% sulfonate solution gave protection for over 145 hours. Additions of 0.5% or 1% to the 5% sulfonate solution gave full protection for over 168 hours. This oil without any sulfonate or ether alcohol permitted rusting within two hours under the conditions of test described above.

## Example 5

A 2% solution of strontium petroleum sulfonate of a molecular weight between five hundred and six hundred was made in an oil useful for lubricating aircraft engines, an S. A. E. 60 Pennsylvania oil of 100 V. I. containing an antioxidant, and to different portions thereof was added 0.5% and 1.0%, respectively, of diisobutylphenoxyethoxyethoxyethanol. Both samples gave perfect protection to steel panels in the humidity tests for over 168 hours. The oil by itself permitted rusting to begin after two hours.

In another type of test, there was established the protective value of the compositions here claimed. A 6% solution of the above sulfonate in the above aviation oil was coated on panels which were immersed in synthetic sea water. At the end of two hours, it was found that rusting had begun on these panels. The addition of 0.5% or 1% of diisobutylphenoxyethoxyethoxyethanol in the 6% sulfonate solution provided complete protection of panels coated with such solutions for forty-eight hours, at which time the tests were discontinued. In the same test were panels coated with a composition comprising 2% of the sulfonate and 1% of the same ether alcohol. These were also free of rust at the end of forty-eight hours of immersion in synthetic sea water. The same result may be obtained by the use of n-decyl- or n-dodecyl- or tert.-dodecyl-phenoxyethoxyethoxyethanol in the solutions of petroleum sulfonates in the above oil.

Compositions such as shown above have been used in commercial applications with results which surpassed those indicated by laboratory tests. The practical applications include not only the use of the compositions as lubricating oils in motors but also the use of the compositions to protect metals from both moisture vapor and condensed moisture during use or during storage.

Oils containing petroleum sulfonates and alkylphenoxyethoxyethoxyethanols, when used as motor oils, have the virtue of preventing corrosion of aluminum pistons, brass and bronze parts and fittings, and bearing alloys, as well as iron and steel parts, guarding against attack by moisture which condenses out within motors. Further-

more, the compositions of the invention may be used for the protection of gasoline and compression-ignition engines in temporary or long-term storage with an added advantage that the engine may be run to distribute the compositions through the motor.

We claim:

- 10 1. A composition of matter consisting essentially of 0.5% to 7.5% of an oil-soluble petroleum sulfonate and 0.05% to 3% of an alkylphenoxyethoxyethoxyethoxyethanol having an alkyl group of four to twelve carbon atoms dissolved in a mineral oil having a viscosity of one hundred to fifteen hundred seconds Saybolt at 100° F.
- 15 2. A composition of matter consisting essentially of 0.5% to 7.5% of an oil-soluble petroleum sulfonate having a molecular weight between four hundred and one thousand and 0.05% to 3% of an oil-soluble alkylphenoxyethoxyethoxyethoxyethanol, having an alkyl group of four to twelve carbon atoms dissolved in a mineral oil having a viscosity of one hundred to fifteen hundred seconds Saybolt at 100° F., the percentage of said alkylphenoxyethoxyethoxyethoxyethanol used not exceeding that of the petroleum sulfonate.
- 20 3. A composition of matter consisting essentially of 0.5% to 7.5% of an oil-soluble petroleum sulfonate of about five hundred to about seven hundred molecular weight and 0.05% to 3% of diisobutylphenoxyethoxyethoxyethoxyethanol, the percentage thereof not exceeding that of said sulfonate, dissolved in a mineral oil having a viscosity of one hundred to fifteen hundred seconds Saybolt at 100° F.
- 25 4. A composition of matter consisting essentially of 0.5% to 7.5% of an oil-soluble petroleum sulfonate having a molecular weight between four hundred and one thousand and 0.05% to 3% of an oil-soluble alkylphenoxyethoxyethoxyethoxyethanol, having an alkyl group of four to twelve carbon atoms dissolved in a mineral oil having a viscosity of one hundred to fifteen hundred seconds Saybolt at 100° F., the percentage of said alkylphenoxyethoxyethoxyethoxyethanol used not exceeding that of the petroleum sulfonate.
- 30 5. A composition of matter consisting essentially of 0.5% to 7.5% of an oil-soluble petroleum sulfonate of about five hundred to about seven hundred molecular weight and 0.05% to 3% of diisobutylphenoxyethoxyethoxyethoxyethanol, the percentage thereof not exceeding that of said sulfonate, dissolved in a mineral oil having a viscosity of one hundred to fifteen hundred seconds Saybolt at 100° F.
- 35 6. A composition of matter consisting essentially of 0.5% to 7.5% of an oil-soluble petroleum sulfonate having a molecular weight between four hundred and one thousand and 0.05% to 3% of diisobutylphenoxyethoxyethoxyethoxyethanol, having an alkyl group of four to twelve carbon atoms dissolved in a mineral oil having a viscosity of one hundred to fifteen hundred seconds Saybolt at 100° F.

FRANK J. GLAVIS.

HARRY T. NEHER.

## REFERENCES CITED

40 The following references are of record in the file of this patent:

## UNITED STATES PATENTS

| Number    | Name   | Date          |
|-----------|--------|---------------|
| 2,075,018 | Bruson | Mar. 30, 1937 |
| 2,176,834 | Bruson | Oct. 17, 1939 |
| 2,408,971 | Duncan | Oct. 8, 1946  |